

## UNITED STATES PATENT OFFICE

CLARKE C. MINTER, OF NEW YORK, N. Y.

## PROCESS OF ETCHING GLASS OR THE LIKE.

No Drawing. Application filed May 27, 1921, Serial No. 473,010. Renewed March 2, 1925.

*To all whom it may concern:*

Be it known that I, CLARKE C. MINTER, a citizen of the United States, residing at New York, in the county of New York and 5 State of New York, have invented a certain new and useful Process of Etching Glass or the like, of which the following is a specification.

My invention relates to the etching of 10 glass or the like, and particularly to the etching of comparatively large portions of the surfaces of articles and objects made of glass or the like, such for example, as window glass, electric light bulbs, lamp shades, 15 to produce ornamental effects or diffusion of light transmitted therethrough, and chinaware and porcelain articles to produce ornamental surface effects.

As is well known, the agent most frequently used in the etching of glass is hydrofluoric acid, a comparatively expensive agent and one in the use of which extreme care and precaution are necessary to be observed to avoid injury to the operator. The 25 care and precaution required further increase the cost of the etching operation, the process when carried on commercially and to any substantial extent usually being performed in a specially-prepared chamber.

Etching has also heretofore been done by the forcible projection of sand or like abrading material against the surface to be etched, and this process has the advantage 35 over etching by hydrofluoric acid in the cheapness of the material used and the safety attending its use, but has the disadvantage that special apparatus and machinery are required to produce the blast of the abrading material.

My invention has, among its objects, to provide a process of etching eliminating the disadvantages of the customary processes heretofore mentioned, by the use of an etching agent or material of comparatively little 45 cost, presenting no danger to the operator in its use, necessitating no elaborate or expensive apparatus or machinery, and requiring comparatively little skill in the performance of the process.

These and other objects will appear from a detailed description later to be given of processes illustrating my invention, but it is to be understood that these processes are merely illustrative of my invention and that 55 my invention is not to be limited thereto.

I have discovered that under certain con-

ditions of temperature of the glass or like object to be etched and of the etching agent, a normal or an acid carbonate of an alkali metal may be used as an effective etching 60 agent.

I preferably employ sodium carbonate although I have also found a mixture of sodium and potassium carbonate an effective agent, the addition of the potassium salt—although having the disadvantage of somewhat increasing the cost over the use of the sodium salt alone—having the advantage of permitting a lower temperature at which the etching is effective. The commercial, as distinguished from the chemically pure salts mentioned, may be used.

The range of temperatures, so far as the heating of the carbonate is concerned, should include the fusion point of the salt, 75 and the heat need not extend appreciably above that point.

The process of etching can be performed either at some stage during the manufacture of the glass or other like object when the 80 heat then being utilized in such manufacture can be utilized for this process, or by reheating the object after its manufacture, and in the later instance, the temperature need not be so high as to distort the object. 85 I have found that heating the object to be etched to approximately what is familiarly known in the arts as a dull red heat of glass is a preferable degree of heat, although not an essential degree as the heat 90 may be varied above that temperature or below the same, the etching being possible at as low a temperature of the glass as approximately 300° centigrade.

My invention may be carried out by any 95 of the following illustrative processes:

1. The glass or like object to be etched is heated in an open flame, into which the desired carbonate, for example sodium carbonate in finely divided particles or powder form, is injected at some point below the glass object.

Any suitable apparatus may be used for injecting the sodium carbonate into the flame, such for example as an apparatus providing an air or other fluid pressure for blowing solid material in finely divided particles. I have found an ordinary bottle of appropriate size partly filled with the powdered salt and with a tube extending below the surface of the salt within the bottle, 105 and terminating outwardly in a nozzle, and

the bottle provided with a collapsible bulb for the creation of an air pressure upon the salt, sufficient for the purpose.

The sodium carbonate thus injected into 5 the flame is itself heated by the flame to the required temperature and quickly carried upwardly into contact with the heated surface of the glass, and the particles of the salt attack the glass wherever they come 10 into contact therewith.

In this case, it is to be observed that a single heating medium is utilized to heat both the glass to be etched and the etching agent.

15 The etching action apparently involves a reaction between the sodium carbonate and the silica of the glass with the production of a soluble silicate, sodium silicate, which is removed by washing the glass with water 20 after the same has been cooled, and carbon dioxide which escapes as a gas. Other reactions may possibly be involved, but in any event, the surface of the glass or like article is pitted and roughened and the desired 25 effect produced.

The powdered salt is applied in the manner stated to the surface of the article after its manufacture, in which case its temperature is raised to the required or desired degree, or during some stage of its manufacture when it is at the suitable temperature,—as, for example, between the blowing of the glass and the finishing of the article, or during the annealing of the same. The simplicity of the process renders it particularly applicable to the etching of the article during its process of manufacture, as indicated, and in the application of the process on a commercial scale, the apparatus for blowing the powdered etching agent upon the surface of the article may be located in the line of travel of the article through the various stages of its manufacture.

2. A melt of the desired carbonate or mixture of carbonates, for example, sodium carbonate, or sodium and potassium carbonates, is prepared, the glass or other-like object to be etched is heated to the required or desirable temperature already stated, and then 50 dipped into the melt referred to, withdrawn, set aside to cool, and washed as before.

Having particularly described my invention, what I claim and desire to secure by Letters Patent is:—

55 1. The process of etching glass or the like comprising heating the glass or the like to be etched and directing an alkali salt of carbonic acid in finely divided particles into contact with the surface to be etched.

60 2. The process of etching glass or the like comprising heating the glass or the like to be etched and directing sodium carbonate in finely divided particles into contact with the surface to be etched.

65 3. The process of etching glass or the like

comprising heating the glass or the like to be etched, directing sodium carbonate in finely divided particles into contact with the surface to be etched, cooling the article thus heated and washing its said surface.

70

4. The process of etching glass or the like comprising heating the glass or the like to be etched, heating an alkali salt of carbonic acid to at least the fusion of said salt, and causing contact of said fused salt with the 75 surface of said glass or the like to be etched.

5. The process of etching glass or the like comprising heating the glass or the like to be etched, heating an alkali salt of carbonic acid to at least the fusion of said salt, causing contact of said fused salt with the 80 surface of said glass or the like to be etched, thereafter cooling said article and washing its said surface.

6. The process of etching glass or the like 85 comprising heating the glass or the like to a temperature approximately 300 degrees centigrade or above, heating an alkali salt of carbonic acid to at least the fusion of said salt, and causing contact of said fused 90 salt with the surface of said glass or the like to be etched.

7. The process of etching glass or the like comprising heating the glass or the like to a temperature approximately 300 degrees centigrade or above, heating an alkali salt of carbonic acid to at least the fusion of said salt, causing contact of said fused salt with the 95 surface of said glass or the like to be etched, cooling the article thus treated and 100 washing the said surface.

8. The process of etching glass or the like comprising heating the glass or the like to a temperature approximately 300 degrees centigrade or above, heating sodium carbonate to at least the fusion point of said salt, causing contact of said fused salt with the surface of said glass or the like to be etched, cooling the article thus treated and 105 washing its said surface.

9. The process of etching glass or the like comprising heating the glass or the like in an open flame, and directing an alkali salt of carbonic acid in finely divided particles into said flame into position to be carried 110 upwardly thereby into contact with the surface to be etched.

10. The process of etching glass or the like comprising heating the glass or the like in an open flame, and directing sodium carbonate in finely divided particles into said flame into position to be carried upwardly thereby into contact with the surface to be etched, withdrawing said article from said 115 flame, cooling said article and washing its 120 said surface.

In testimony that I claim the foregoing, I have hereunto set my hand this 26th day of May, 1921.

CLARKE C. MINTER.